

June 13, 1961

A. T. WALTER

2,988,419

PROCESS FOR SPINNING AND DRYING FIBERS OF A POLYMER CONTAINING  
A SIGNIFICANT AMOUNT OF ACRYLONITRILE POLYMERIZED THEREIN  
Filed Jan. 18, 1957

2 Sheets-Sheet 1

*Fig. 1.*



*Fig. 2.*



*Fig. 3.*

INVENTOR  
ANDREW T. WALTER

BY  
*Frank Smith*  
ATTORNEY

June 13, 1961

A. T. WALTER

2,988,419

PROCESS FOR SPINNING AND DRYING FIBERS OF A POLYMER CONTAINING  
A SIGNIFICANT AMOUNT OF ACRYLONITRILE POLYMERIZED THEREIN

Filed Jan. 18, 1957

2 Sheets-Sheet 2



Fig. 4.



Fig. 5.

INVENTOR  
ANDREW T. WALTER

BY *John Smith*  
ATTORNEY

# United States Patent Office

2,988,419

Patented June 13, 1961

1

2,988,419

## PROCESS FOR SPINNING AND DRYING FIBERS OF A POLYMER CONTAINING A SIGNIFICANT AMOUNT OF ACRYLONITRILE POLYMERIZED THEREIN

Andrew T. Walter, Charleston, W. Va., assignor to Union

Carbide Corporation, a corporation of New York

Filed Jan. 18, 1957, Ser. No. 634,888

9 Claims. (Cl. 18—54)

This invention relates to a process for producing continuous filament textile yarns and tow of uniform composition and low solvent content from vinyl polymers. More particularly, this invention relates to an improved continuous process for producing continuous filament yarns and tow containing less than 2 percent of residual solvent from an acrylonitrile-containing polymer without cementation or undesirable effect on the spun fibers.

It is generally known that vinyl polymers, particularly those containing a substantial amount of acrylonitrile can be wet or dry spun into continuous filament yarns and tow useful in producing textile products for industrial, apparel, and household applications. In spite of their recognized utility, commercial production is currently quite small compared with staple fiber or heavy tow made from these same polymers. This situation is unlike that found with most other man-made fibers where filament yarns constitute a large portion of total fibers produced.

A major reason that filament yarns produced from acrylonitrile polymers have not attained a relatively large scale commercial production is due to the technological difficulties and associated high costs encountered in manufacturing. These problems in a large part are attributable to the difficulty of removing residual solvent from the yarn after it is spun by presently employed techniques. Under dry spinning techniques, the fiber will emerge from the spinning tube containing about 10 percent to 20 percent residual solvent. In wet spinning, a solution of the resin in a volatile spinning solvent is extruded into a coagulant or extractant bath which is a non-solvent for the resin but which is miscible with the spinning solvent and removes most of the residual solvent from the resin. Amounts of 10 to 20 percent of residual spinning solvent in the fiber are nevertheless usually encountered. It is obvious that the solvent content of such fibers must be reduced before they can be made useful for textile applications.

During the spinning operations, the fibers take on a comparatively hard and impervious surface after the solvent content is reduced to 10 to 20 percent of the weight of the fiber, greatly impeding further removal of solvent by slowing diffusion of solvent to and through the surface. The rate of solvent loss is therefore markedly reduced. From this point on, heretofore it has been very difficult to remove additional solvent unless extended drying periods at high temperature or prolonged extraction in a liquid medium are employed. The use of temperature necessary to remove the greater part of the residual solvent within several minutes invariably causes surface fusion and cementation of adjacent filaments, making the yarn unsuitable for most applications. Drying periods of several hours duration at temperatures considerably below the fusion or cementation temperature are required to reduce the solvent content of the fiber to the desired level (below two percent by weight and preferably less than one percent). Drying periods of such a magnitude are objectionable and cannot be accommodated in continuous filament yarn processes, which depend upon high spinning speeds and short processing times. Heretofore, the processes had to be discontinuous in that the filament formation and solvent-removal steps

2

had to be carried out separately in the manufacture of the yarn, and such other steps as orientation and annealing also had to be carried out separately. This required the handling and storage of a great many packages or bobbins of yarn during the manufacturing operation and often resulted in several hours, or even days, elapsing between the time the spinning solution was forced through the spinneret and the time a finished solvent-free yarn was produced.

- 10 The dyeing characteristics of the fibers are profoundly affected by slight variations in the amount of residual solvent. It is essential that the solvent content of the fiber be maintained within very close limits if satisfactory uniformity of dyeing is to be achieved and "barre effect" in textiles made therefrom is to be eliminated. As a practical matter, it is nearly impossible to control solvent content with the necessary precision at any level above about 2 percent—hence it is necessary in practice to maintain the solvent content of the fiber at a low final value, i.e. less than two percent, in order to obtain satisfactory dyeing uniformity. As indicated, non-continuous processes are employed in actual practice. In most commercial applications the newly spun fibers are wound on bobbins and back-flushed for several hours in a hot water bath or loaded into drying ovens for extended periods at elevated temperatures to drive off the solvent. Such non-continuous processes are not only time-consuming and costly, but also it is virtually impossible to operate such noncontinuous processes without introducing serious non-uniformity into the yarns, particularly in continuous filament yarn production. Thus, if a given lot of yarn that contains for example about 15 percent of solvent, is stored for even a brief period on a bobbin or reel, the solvent content of the yarn on the outside of the package will soon be different from that of the yarn on the inside of the package. The yarn from the two locations will therefore respond quite differently to the tensions that are imposed in subsequent processing operations, and non-uniform fibers will result. In addition, these fibers will possess different dye absorption characteristics in a standard dye bath, creating variations in shades of the desired color which, when the fibers, are formed into fabrics, becomes rather pronounced, imparting thereto a "barre effect." For these reasons, the present method for continuously and quickly producing a fiber of uniform composition containing less than two percent of residual solvent content is highly advantageous.
- 15
- 20
- 25
- 30
- 35
- 40
- 45

According to the present invention, I have now discovered an improved solvent spinning process for continuously producing lustrous, void-free textile filaments, fibers, and yarns having uniform residual solvent content of less than 2 percent in less than about three minutes from a solution of a vinyl resin in a volatile spinning solvent. The process of this invention includes the steps of extruding a dope composed of a vinyl polymer dissolved in a volatile spinning solvent boiling below about 100° C. through a spinneret to form fibers containing about 20 percent by weight or less of residual solvent, subjecting the formed fibers to direct contact with a heated surface having a surface temperature of at least about 60° C. and between 5° C. and 20° C. below the fusion temperature of the fibers at the point of contact with the heated surface, increasing by increments the temperature of the surface with which the moving fiber is in contact at a rate such that the fiber-contacting surface temperature is maintained at least 5° C. below the fusion temperature of the fiber at such contacting points to a final surface temperature between 135° C. and 190° C. and until said fibers have a residual solvent content of less than 2 percent by weight and a fusion temperature of at least 150° C.

By the term "fusion temperature" as used herein, I

mean the critical temperature at which the contacting fibers become tacky and stick together, i.e. the temperature at which two or more filaments of a multifilament yarn, strand, or tow become fused or adherent to each other to such an extent that they are difficult or impossible to separate by normal methods of handling, such as by passing the fibers over guides and flexing with tensions normally encountered. This interfiber bonding or fusion can readily be identified by microscopic inspection, and is evidenced by a pronounced stiffening of the yarn. The temperature at which the interfiber fusion takes place is influenced by the pressure or tension applied to the yarn in a manner such that the fusion temperature of the fiber decreases as tension is increased, such as is shown in FIGURE 1. A convenient correlation of fusion temperature and shrinkage of the fibers exists so as to give an estimation of fusion temperature. I have found that within normal limits of error, the fusion temperature of the fiber will be about the temperature at which the fiber will shrink about 50 percent under no tension.

The fusion temperature should not be confused with the temperature necessary to reluster or fuse the interior of the fiber. The relustering temperature (or interfiber fusion temperature) of a fiber will be lower than the exterior fusion or interfiber bonding temperature. This relustering temperature can vary from several degrees to 20° C. or more below the interfiber fusion temperature because of the normally higher solvent content in the interior of the fiber.

As an embodiment of this invention, the solvent removal from the fiber is combined with a simultaneous relustering of the fiber over a temperature range that corresponds to the change in fusion temperature of the fiber as the solvent content of the fiber is reduced. At the beginning of the solvent removal from the fiber when the fiber is most susceptible to fusion or cementation, a low temperature of the fiber contacting surface is necessary. The initial temperature must be at least 60° C. and may range from about 60° C. to about 120° C. but always between 5° and 20° below the fusion temperature of the fiber at that point. As solvent removal proceeds, the fiber contacting surface temperature is increased, either continuously in minute increments or in a step-wise manner of several larger steps to a maximum temperature which ranges between about 135° C. and 190° C. but always at least 5° C. below the fusion temperature of the fibers at the contact point.

In carrying out this invention, I have found that the most convenient way of securing and maintaining such critical temperature control is by means of heated rolls or godets. The heating can be by internal or external means as desired. In order to secure this increasing temperature gradient during the solvent removal from the fiber, a series of rolls or godets may be employed, each succeeding one heated to a higher temperature than the preceding, and controlled as to be within the limits as hereinbefore set forth. As an alternative, two long rolls arranged on non-parallel axes (a godet) may be employed such as to have an increasing temperature gradient maintained along its axial length, with either one or both rolls being heated and/or driven. Multiple laps of the fibers about these rolls will enable the fibers to be gradually heated without suffering fiber fusion as they advance from the cooler to warmer sections of the rolls. Similar results can be obtained if only one of two long rolls is heated and the second roll of the godet merely serves as an idler roll to facilitate the advancement of the yarn from the cooler to the hotter end of the heated roll.

A particularly desirable method for achieving the temperature gradient on the heated roll or rolls is to so construct them as to be internally heated on one end by steam coils or jacket or electrical resistance wire. The unheated end of the roll would then be maintained

at a temperature somewhat below the temperature of the heated end by conducted heat. By having the fibers first contact the unheated end of the roll, and with many turns about the roll, solvent removal can proceed such that the fibers upon reaching the heated end can withstand the increased heat without fusion. Two such internally heated godets might also be arranged in series to achieve a greater overall temperature gradient.

By maintaining the heated surface or roll at a temperature close to, but at least 5° C. below, the fusion temperature curve, substantially solvent-free fibers can be achieved in less than three minutes. I have found it possible to produce a fiber having about 0.15 percent by weight or less of residual solvent in the fiber in less than three minutes and often within one minute total drying time. This is particularly desirable in continuous filament yarn production where spinning speeds must be quite high in order to achieve a reasonable poundage per hour of continuous filament yarn. By following the practice of this invention, no slow-down in production is necessary for removing solvent from the fiber. In fact, such continuously produced yarn can go directly into further processing steps without storage and collection on bobbins.

The fusion temperature of the fibers is sharply dependent both on solvent content and on the acrylonitrile content of the polymer. Solvent present in the fibers, even in modest quantities, has a plasticizing effect on the fiber and profoundly reduces the fusion temperature. For instance, a solvent-free copolymeric fiber containing 40 percent acrylonitrile and 60 percent vinyl chloride has a fusion temperature of about 150° C., but a freshly spun fiber of this composition containing about 15 percent by weight residual solvent shows a fusion temperature of about 70° C. Similarly, a nearly solvent-free polymer containing 70 percent acrylonitrile and 30 percent vinyl chloride has a fusion temperature of about 240° C., but the freshly spun fiber containing about 15 percent by weight of solvent has a fusion temperature of about 90° C. to 100° C. A similar increase in fusion temperature with an increase in acrylonitrile content is noted with other acrylonitrile-containing polymers.

In all cases with these vinyl polymers the fusion temperature increases with a decrease in solvent content in a manner similar to that shown graphically in FIGURE 1. This figure illustrates variations of fusion temperature with changes of the residual solvent content of a representative terpolymer resin fiber containing 68 percent acrylonitrile, 21 percent vinyl chloride, and 11 percent vinylidene chloride using acetonitrile as a spinning solvent, under both low and high tension (low tension being about 0.01 gram per denier and high tension being about 0.1 gram per denier). As can be readily seen from FIG. 1, freshly spun fibers containing 15-20 percent of the spinning solvent have a low fusion temperature, i.e. about 65° C. to 100° C. but as the solvent content is reduced the fusion temperature of the fiber increases to about 250° C. It is my purpose in this invention to carry out the solvent removal and relustering at temperatures following as closely as possible this fusion temperature curve.

Vinyl polymers and copolymers in which at least one component is acrylonitrile polymerized therein and which can be spun from spinning solvents boiling below 100° C. into a fiber having a solvent-free fusion temperature of at least 150° C. can be employed in the practice of this invention. Preferred of these vinyl polymers are polymers containing a substantial amount of acrylonitrile, particularly the polymers containing between 40 and 75 percent acrylonitrile and 25 to 60 percent of another polymerizable vinyl composition such as vinyl chloride, vinyl acetate, vinylidene chloride, and the like. Particularly desirable results are achieved on the terpolymer composition shown for FIGURE 1, spinning from an acetonitrile solvent. Good results are also achieved with a

40 percent acrylonitrile—60 percent vinyl chloride copolymer and with copolymers containing 60 to 70 percent acrylonitrile and 30 to 40 percent vinyl chloride or vinylidene chloride.

It is not critical in the operation of this process that the fibers be initially formed in any particular manner. The process is applicable to wet spinning into a liquid coagulant such as water or a water solvent mixture, or to dry spinning methods wherein the fibers are extruded into a stream of heated gaseous medium such as air or steam in a tube or chimney. It is necessary, however, that the coagulant bath or heated gaseous medium be able to remove sufficient solvent from the fiber to permit fiber contact without fusing. This is possible with a fiber having about 20 percent or less of residual solvent content in the fiber.

Under the conditions of operation as herein set forth, the solvent content of freshly spun fibers can be rapidly reduced from an initial value of about 20 percent to less than 2 percent within three minutes or less. Such rapid solvent removal is not possible by other known methods and makes it possible for fibers to be continuously spun, stretched, annealed, lubricated, twisted, and wound up on a finished package. The process is particularly desirable for continuous filament yarn production where high spinning speeds are employed. In continuous filament yarn production the number of filaments is quite low, generally about 250 or less, and high spinning speeds are necessary to produce an appreciable poundage of yarn per day. Thus continuous movement of the fibers and yarns from the spinning through the drying, orientation, and annealing operations is highly desirable. The fibers thus produced are characterized by a high degree of uniformity as to diameter and solvent content and are suitable for all subsequent processing operations. The uniformity of yarn achieved by this method greatly reduces "barre effect" in dyed fabrics made therefrom.

This process can best be illustrated by reference to the attached drawings. FIGURE 1 shows the hereinbefore discussed relationship of solvent content to fusion temperature of the fiber. FIGURE 2 represents one of the preferred forms of carrying out the invention by the use of two internally heated advancing rolls having intersecting axes in which the gradual increase in temperature is maintained in an increasing gradient across the rolls. FIGURE 3 illustrates a form of the invention particularly applicable to the continuous spinning of a heavy fiber tow, using a series of seven heated rolls, each at a temperature above the previous roll but below the fusion temperature of the fiber. FIGURE 4 shows the process as applied to dry spinning techniques employing a series of three heated rolls in combination with a stretching and annealing device. FIGURE 5 illustrates a permissible modification employing a fiber pre-wash in connection with two heated advancing rolls followed by stretching and annealing.

The process of FIGURES 2, 3, 4, and 5 diagrammatically illustrates several methods of carrying out this invention. In reference to FIGURE 2 illustrating one of the preferred forms of apparatus useful in practicing the invention, spun fibers are formed by metering the polymer solution through spinneret 2 into a bath 1 containing a liquid that is miscible with the solvent but which is a non-solvent for the fiber polymer, generally water. Sufficient solvent is removed from the yarn so that the filaments can be drawn together without fusing or sticking to each other. The yarn is then drawn over a guide pin or roll 3 and withdrawn from the bath and wrapped around the low temperature end of the heated advancing rolls 4 and 5 with 30 to 100 turns in a helical path so that the yarn is heated and solvent removed without fusing the filaments for a total residence period of two minutes or less on the rolls. The rolls are internally heated to a temperature of at least 60° C. at the low temperature end, with the interior of the rolls heated with steam such that an increasing temperature gradient

is maintained across the rolls to a final temperature between 135° C. and 170° C.

The nearly solvent-free yarn leaving rolls 4 and 5 can be wound on a suitable winding device 9 or, as shown, 5 can be stretched on stretching wheel 6 through heater 7 with a relaxation of tension on wheels 8 to anneal the fiber.

In FIGURE 3, the polymer solution is forced through 10 a spinneret 12 below the surface of the coagulating medium in bath 11 withdrawn from the bath over pin 13 and, if desired, lubricant applied by a suitable applicator 14 and fed to a series of identical drying rolls 15a to g. The first of these rolls, 15a, is maintained at a temperature of at least 60° C. and between 5° and 20° C. below the 15 fusion temperature of the fiber. Each subsequent roll 15b to g is maintained each at increasing temperatures to a final temperature between 135° C. to 170° C., with the fibers, preferably a tow of 1000-2500 individual fibers, 20 making less than a complete lap on each heated roll, and wound up on a take-up bobbin 16.

In FIGURE 4, the yarn is dry-spun through a hot air 25 drying tube 21 from spinneret 22 through a counter-current stream of hot air. The yarn issuing from the bottom of the tube will contain about 10-15 percent of 30 residual solvent. Lubricant can be applied to the yarn by a suitable applicator 23, and the yarn dried on a series of three drying godets 24, 25, and 26. The temperature of 25 being higher than 24, and the temperature of 26 being higher than 25. Each godet can, if desired, 35 have an independent temperature gradient across the roll as hereinbefore described. The nearly solvent-free yarn can be directly processed by stretching steam tube 27 and godet 28, and annealing with a suitable annealing device 29 and tensioning godet 30 and picked up on a bobbin or winding device 30a.

Another form of the practice of this invention is illustrated in FIGURE 5. The polymeric solution is forced through spinneret 31 into the coagulating medium in bath 32 and withdrawn from the bath over pin or roller 33. 40 The fiber can be washed with water or solvent in a suitable device 34 and 35 to wash off the spinning bath "carry out" or to further extract spinning solvent from the fiber to reduce solvent content to less than 20 percent. The fibers are then conducted over the first heated advancing godet 36 with sufficient laps so that solvent content is reduced to about 4-5 percent and then conducted to a second heated advancing godet 37 where the solvent content is reduced to less than 2 percent. Stretching is 45 accomplished by godet 38 and annealing in device 39 and godet 40 and the fiber taken up on a suitable take-up bobbin 41.

The following examples are illustrative. When herein 50 employed the word "yarn" means the bundle of fibers containing one filament for each spinneret hole.

#### Example 1

Twelve pounds of a copolymer consisting of 33.6 percent vinyl chloride and 66.4 percent acrylonitrile having a specific viscosity of 0.347 at 20° C. in a 0.2 percent 60 solution of dimethylformamide were added to 48 pounds of acetonitrile contained in a jacketed dope-mixing pot at room temperature. The slurry was heated with stirring until solvated and the pot sealed and heating was continued for one hour at 90° C. The solution was cooled to 75° C., filtered, and metered to a spinneret containing 1250 holes, each 0.14 mm. in diameter. The filaments were extruded at the rate of 10-15 ft./min. into a coagulating bath consisting of a mixture of water and acetonitrile in a weight ratio of 85-to-15 maintained at 65° C., and then passed to a second bath consisting of water maintained at 85° C.-95° C. After about one minute contact in the baths, the yarn was withdrawn from the bath and passed onto the first of a series of four drying wheels or drums. Each wheel was 3 feet in diameter 70 and 4 inches wide and was heated by means of steam and 75

circulated through tubing welded to the inside circumferential surface of the wheel. The temperature of the outside surface was controlled separately for each wheel by adjusting the steam pressure in the tubing. The surface temperature was lowest for the first wheel maintained between 5° C. and 20° C. below the fusion temperature of the fiber in order to avoid filament fusion and was increased progressively with each succeeding wheel. The wheels were arranged as shown in FIGURE 3 so that the yarn was carried approximately two-thirds around each wheel before progressing to the next wheel. The wheels were rotated with a surface speed of 16.5 ft./min. to provide a total drying time of 103 seconds, or about 26 seconds for each wheel. The dry weight of the yarn (less all water and solvent) was determined at various points in the drying operation by measuring the loss in weight of yarn skeins after drying for 30 minutes at 125° C., conditions which are known to remove all volatile material. The freshly spun yarn after leaving the bath and before contacting the first drying wheel containing about 13 percent solvent retained in the fiber and about 120 percent excess coagulant carried out of the bath on the surface of the yarn.

A large portion of the liquid or volatile material was removed from the yarn on the first wheel and the remainder was removed on the subsequent wheels. The percent total solids (percent dry weight) of the yarn after contacting each wheel and the surface temperature of each wheel is given in the following table.

| Drying Wheel | Drying Wheel, °C. | Percent Total Solids of Yarn After Contacting Drying Wheels |
|--------------|-------------------|-------------------------------------------------------------|
| No. 1.....   | 113               | 173.0                                                       |
| No. 2.....   | 122               | 178.0                                                       |
| No. 3.....   | 127               | 96.0                                                        |
| No. 4.....   | 136               | 98.8                                                        |

<sup>1</sup> Including coagulating bath liquid carry-out on fibers.

After the fourth drying roll, the volatile solvent content, corresponding to the amount of solvent still retained in the yarn, was reduced to a value of only 1.2 percent of the total weight of the dried yarn. This was accomplished in less than two minutes without fusing the filaments of the yarn. The dry yarn was then stretched 900 percent in a steam stretching tube heated to about 120° C., annealed by allowing 16 percent shrinkage while passing through a slotted bar heated to 205° C., and then was wound on a spinning bobbin. The resulting 3875-denier, 1250-filament yarn had a tenacity of 3.16 grams per denier, 17.5 percent elongation at break, and 1.8 percent and 1.6 percent shrinkage in boiling water and 150° C. air, respectively. It was lustrous, void free, and had a soft and open feel free of fiber fusion.

#### Example 2

A spinning solution consisting of 150 parts of acetonitrile, 50 parts of an acrylonitrile-vinyl chloride copolymer (69.1 percent acrylonitrile, 30.9 percent vinyl chloride, specific viscosity of 0.442 at 20° C. in dimethylformamide) and 1 part of diethyl tin maleate as a stabilizer was prepared by making a slurry at room temperature and then heating to about 80° C. to bring about the dissolution of the resin in one hour. The solution was then pumped at 75° C. through a spinneret having 40 holes, each 0.10 mm. in diameter, at a rate of 12.5 cc. per minute. The yarn was coagulated by passing upward through a bath containing 9 parts by weight of water to 1 part of acetonitrile at 75° C. for a distance of about 30 inches. The yarn was withdrawn from the bath by an unheated godet located immediately above the bath, and then advanced in a helical path around the godet with ten laps while being washed with a stream of water at 92° C. flowing at a rate of 180 cc. per minute. The coagulated and washed yarn containing 15.9 percent sol-

vent by analysis was then passed to drying rolls consisting of two rolls, 4 inches in diameter and 24 inches long. The rolls were located one over the other with their axes intersecting in a common plane as shown in FIGURE 2 so that the yarn was made to pass 80 times in a helical path around the two rolls as it advanced from one end to the other. Both rolls were heated internally in four separate sections so that the temperature of each roll could be increased from one end to the other. By this method the yarn was first subjected to a low drying temperature at the initial contact and then to increasing temperatures as it advanced across the godet. The surface temperature at various points along the roll, the time required for the yarn to advance to this point, and the solvent content of the yarn at each point are summarized in the following table.

|         | Distance yarn advanced across godet, inches | Approximate time required for yarn to advance, sec. | Temperature of godet at the point of yarn advance, °C. | Solvent retained in yarn at point of advance, percent |
|---------|---------------------------------------------|-----------------------------------------------------|--------------------------------------------------------|-------------------------------------------------------|
| 0.....  |                                             | 0                                                   | 102                                                    | 15.9                                                  |
| 5.....  |                                             | 25                                                  | 114                                                    | 8.3                                                   |
| 10..... |                                             | 45                                                  | 131                                                    | 4.9                                                   |
| 15..... |                                             | 60                                                  | 138                                                    | 3.5                                                   |
| 20..... |                                             | 95                                                  | 162                                                    | 1.8                                                   |

The data in the above table show that the solvent content was reduced to less than 2 percent in only 95 seconds drying time. The drying operation was also accomplished without causing filament fusion. The yarn was soft and open, lustrous, and void free and was suitable for further processing such as stretching and annealing.

By way of contrast, a similar yarn sample was coagulated and washed in a similar manner and wound around the same drying godet that was instead heated to a uniform temperature of 105° C. This was the highest temperature that could be used without causing serious filament cementation, and after the yarn had advanced across the godet for approximately 20 inches—in this case requiring 105 seconds—it still contained as much as 4.5 percent solvent by analysis. Therefore, in spite of the slightly longer drying time, the solvent content could not be reduced to an acceptable value by employing a fixed drying temperature.

#### Example 3

Seventeen hundred and twenty-four grams (1724) of a terpolymer consisting of 69.6 percent acrylonitrile, 20.4 percent vinyl chloride, and 10.0 percent vinylidene chloride having a specific viscosity of 0.368 at 20° C. in an 0.2 percent dimethylformamide solution, 26 grams of diethyl tin maleate and 5250 grams of acetonitrile were slurried in a jacketed dope mixing pot. The slurry was heated to 70° C. and mixed until solvation occurred. The vessel was sealed and the temperature increased to 83° C. and maintained at that temperature during the entire spinning operation. The solution was then pumped through a dope filtering system to a metering pump that metered the dope to a spinneret having 100 holes each 0.16 mm. in diameter. The solution was extruded at a rate of 23 cc. per minute into a bath consisting of water and acetonitrile in the ratio of 85 to 15 at 64° C. through a distance of 45 inches. The freshly coagulated yarn containing about 17.3 percent residual solvent, and having a fusion temperature of about 100° C. was withdrawn from the bath and passed continuously at a rate of 94 ft. per minute around a godet consisting of an unheated idler roll 10 inches long and 1.5 inches in diameter, and a heated drying roll 10 inches long and 8.5 inches in diameter.

The roll was internally heated with steam to a temperature of 110° C. but due to the evaporation of water from the yarn and the relatively low heat transfer of the roll, the surface temperature was reduced to 90° C. at the

point where the yarn first contacted the roll. The yarn made approximately 33 laps on the godet, advancing in a helical path from the cool (90° C.) end of the roll to the warm end (110° C.) with a period of 53 seconds. At this point the water was completely evaporated from the surface of the yarn and the residual solvent content was analyzed and found to be 5.1 percent and had a fusion temperature of about 185° C. This yarn, which was then very much more resistant to filament fusion than the freshly coagulated yarn was passed to a second heated godet similar in construction to the first godet, but heated to a surface temperature of 187° C. and rotating at a rate of 100 ft. per minute. The yarn made 25 laps around the hot godet as it advanced in a helical path to the forward end of the roll within a period of 37 seconds.

The yarn was stretched 522 percent at 187° C. by means of a stretching godet operating at a speed of 622 ft. per minute. After about four laps around the unheated stretching godet, the yarn was passed continuously through an annealing device where the yarn was heated to a temperature of 220° C. for approximately 0.02 seconds and allowed to shrink 11.2 percent. The stretched and annealed yarn containing only 0.15 percent residual solvents by analysis was wound up on a spinning bobbin at 560 ft. per minute. The yarn was lustrous and void free, and had a soft feel and the individual filaments in the yarn could easily be distinguished from each other indicating that the yarn was unfused. The finished yarn was produced with a total process time of only about 95 seconds and at a spinning rate of approximately 0.4 pounds per hour.

The properties of the 209-denier, 100-filament yarn obtained in the above described manner were as follows:

|                                    |      |
|------------------------------------|------|
| Tenacity, g.p.d. -----             | 3.74 |
| Elongation at break, percent ----- | 16   |
| Percent shrinkage in:              |      |
| Boiling water -----                | 2    |
| 150° C. air -----                  | 1    |
| 200° C. air -----                  | 5.5  |

#### Example 4

Fourteen hundred and seventy-eight grams of a copolymer consisting of 67 percent acrylonitrile and 33 percent of vinyl chloride having a specific viscosity of 0.251 at 20° C. in an 0.2 percent dimethylformamide solution, together with 23 grams of dioctyl tin maleate and 4500 grams of acetonitrile were slurried in a jacketed dope mixing pot. The slurry was heated to 70° C. and mixed until solvation occurred. The vessel was sealed and the temperature increased to 83° C. The solution was then pumped through a filtering system to a metering pump that metered the dope to a spinneret having 100 holes each 0.16 mm. in diameter. The solution was extruded at a rate of 23 cc. per minute into a bath consisting of water and acetonitrile in a weight ratio of 87.5 to 12.5 at 65° C. and traveled through the bath for a distance of 45 inches. The freshly spun yarn, which was analyzed and found to contain 15.4 percent residual solvent, having a fusion temperature of about 100° C. was then drawn continuously from the bath and passed to an internally heated godet at a rate of 94 ft. per minute in a manner similar to that described in Example 5. The wet yarn first contacted the roll at a roll temperature of 90° C. and made 40 laps around the godet as it advanced to the forward end of the roll within a period of 66 seconds. The surface temperature of the roll contacting the yarn gradually increased to 112° C. as the water was evaporated from the surface of the yarn, and the yarn leaving this roll contained 5.8 percent residual solvent by analysis and had a fusion temperature of 205° C. The yarn was then passed to a second heated godet operating at 100 ft. per minute and 170° C. upon which it advanced in 23 laps to the forward end of the roll within a period of 35 seconds. The yarn was then dry-stretched 522 percent over a heated stretching wheel

75

attached to the second drying godet. The stretched yarn contained only 0.7 percent residual solvent. It was then passed continuously through an annealing device at 220° C. wherein it was heated to about 220° C. for approximately 0.02 second and was allowed to shrink 10.2 percent. The 211-denier, 100-filament stretched and annealed yarn containing 0.7 percent residual solvent was wound up at a rate of 550 ft. per minute and upon examination showed a lustrous, void free appearance, free from filament fusion. The properties of the yarn produced in this manner are summarized below.

|                                    |          |
|------------------------------------|----------|
| Final fusion temp. -----           | >250° C. |
| Tenacity, g.p.d. -----             | 3.45     |
| Elongation at break, percent ----- | 17.0     |
| Percent shrinkage in:              |          |
| Boiling water -----                | 3.0      |
| 150° C. air -----                  | 3.0      |
| 200° C. air -----                  | 10.0     |

#### Example 5

Two thousand grams of a copolymer consisting of 60.2 percent vinyl chloride and 39.8 percent acrylonitrile and having a specific viscosity of 0.26 at 20° C. in an 0.20 percent solution of cyclohexanone, together with 40 grams of dioctyl tin maleate were added to 5140 grams of acetone at -20° C. to form a slurry. The slurry was heated while stirring in a jacketed vessel to 45° C. whereupon the slurry became very viscous due to solvation of the resin. The vessel was sealed and the temperature increased to 80° C. After one hour at 80° C., the temperature of the solution was reduced to 50° C. and was then pumped through a filter and fed to a gear-type metering pump. The solution was metered to a spinneret consisting of 500 holes each 0.15 mm. in diameter, and extruded at the rate of 45 feet per minute into a coagulating bath consisting of water and acetone in a weight ratio of 85-to-15 at 50° C. After a coagulation period of 5.4 seconds, the freshly coagulated yarn was withdrawn from the coagulation bath and passed around a godet where it was washed for a period of 5 seconds with water at about 60° C. The yarn was then passed to the first drying godet consisting of an unheated idler roll 10 inches long and 1.5 inches in diameter and an internally heated roll 10 inches long and 8.5 inches in diameter turning with a peripheral speed of 47.8 feet per minute and a maximum surface temperature of 52° C. The yarn advanced in a helical path around the godet with a sufficient number of laps to provide a total heating time of about 135 seconds. After leaving the first drying godet, the surface of the yarn was dry and enough of the residual solvent in the yarn was removed to permit it to be further dried at a much higher temperature without encountering fusion of the filaments in the yarn. The yarn was thus passed to a second drying godet similar in construction to the first but heated internally to a surface temperature of 140° C. The yarn advanced in a helical path around the godet with 29 laps to provide a contact time of 85 seconds. After the drying was completed, the hot yarn was stretched 350 percent directly from the surface of the drying roll by means of an unheated stretching godet operating with a surface speed of 222 feet per minute. The stretched yarn was later annealed in a separate operation by passing it through a slotted bar heated to about 150° C. at a rate of 200 feet per minute. The yarn was heated by radiation for approximately 5 seconds, and during this period was allowed to shrink 10 to 12 percent.

The final 3372-denier, 250-filament yarn was soft and "open" which indicated that it was free of filament fusion, and by analysis had only from 1.3 to 1.5 percent residual acetone and was lustrous and void-free. Solvent content of the tow was measured by extracting the solvent from the yarn for 16 hours in water in 100° C. and then analyzing the extractant for acetone content. The physical properties of the annealed yarn are: denier, 3372; tenacity, g.p.d., 1.7; elongation at break, percent 70.0; percent

shrinkage in boiling water, 5.0; in 125° C. air, 4.5; and in 150° C. air, 49.0.

*Example 6*

A two inch, 3 denier staple fiber of a 60 percent acrylonitrile-40 percent vinylidene chloride copolymer, manufactured by the Tennessee Eastman Company under the name of Verel was scoured in a soap solution at 50° C. to removing processing finishes, rinsed in 50° C. water and dried at 65° C. in a circulating air oven for 16 hours.

Seven hundred and seventy-five grams (775) of the above scoured fiber which had a specific viscosity of 0.238 in a 0.2 percent dimethylformamide solution at 20° C. were mixed with 3000 grams of acetonitrile and heated to 50° C. for one hour to form a solution. Evaporation losses were such as to reduce the acetonitrile content to 1938 grams. The jacketed mixing vessel was sealed and the solution aged for one hour at 80° C. to remove bubbles. The solution was then pumped through a filtering system to a metering pump and thence through a spinneret having 100 holes each 0.10 millimeter in diameter. The solution was extruded at a rate of 83.5 feet per minute into an aqueous coagulating bath containing 10 percent acetonitrile at 60° C. The yarn was withdrawn from the bath after 2.7 seconds by a godet located immediately above at a rate of 83.5 feet per minute and advanced in a helical path with eight laps around the godet for 8 seconds while being washed with an aqueous solution at 82° C. containing 0.5 percent polyoxyethylene glycol having an average molecular weight of about 4000. The washed yarn which contained 7.10 percent solvent by analysis was then passed continuously at a rate of 97 feet per minute onto an internally heated godet whose surface temperature at this end was 113° C. The yarn advanced in a helical path for 29 laps to provide a contact time of 52 seconds. The surface temperature of the godet at this point was 126° C. After leaving the first drying godet the yarn contained 2.49 percent solvent by analysis and was continuously passed to a second internally heated godet having a surface speed of 102 feet per minute and a surface temperature at this end of 142° C. After 29 laps, or a contact time of 43 seconds, the yarn containing 0.94 percent solvent was withdrawn from the drying godet at a point where the surface temperature was maintained at 164° C. The dry yarn passed continuously to a stretching godet operating at a surface speed of 612 feet per minute to induce a stretch of 500 percent. From this godet the yarn passed through an annealing device heated to about 230° C. wherein the yarn was exposed for about 0.2 second and allowed to shrink 15.2 percent and was finally wound onto a spinning bobbin at 519 ft. per minute. By this method yarns essentially free of solvent (less than 1.0 percent by analysis) were produced which were lustrous and free of voids and interfiber fusion. Properties of continuously produced 265 denier, 100 filament yarns are summarized below.

|                                    |      |
|------------------------------------|------|
| Dry tenacity, g.p.d.               | 2.4  |
| Elongation at break, percent       | 11.0 |
| Percent shrinkage in boiling water | 8.0  |

I claim:

1. A process for continuously producing textile filaments and yarns having low solvent content and free from interfiber fusion from a vinyl polymer in which at least one component is acrylonitrile present in a significant amount polymerized therein, which includes the steps of extruding a dope consisting of the said polymer dissolved in a spinning solvent boiling below about 100° C. through a spinneret to form fibers containing less than about 20 percent by weight of residual solvent and subjecting the formed fibers to direct contact with a heated surface maintained at a temperature of at least about 60° C. and between 5° C. and 20° C. below the fusion temperature of the fiber at the point of contact with the heated surface, increasing by increments the temperature of the surface to which the fiber is in contact at a rate such that the fiber contacting surface is maintained at least 5° C. below the fusion temperature of the fiber at such contacting points to a final surface temperature between 135° C. and 190° C. and until said fibers have a residual solvent content of less than about 2 percent by weight and a fusion temperature of at least 150° C.

5 2. A process for continuously producing textile filaments and yarns having low solvent content from a vinyl polymer containing between about 40 percent and about 75 percent acrylonitrile polymerized therein, which includes the steps of extruding a dope consisting of the said polymer dissolved in a spinning solvent boiling below about 100° C., through a spinneret to form fibers containing less than about 20 percent by weight of residual solvent, and subjecting the formed fibers to direct contact with a heated surface maintained at a temperature of at least about 60° C. and between 5° C. and 20° C. below the fusion temperature of the fiber at the point of contact with the heated surface, increasing by increments the temperature of the surface to which the fiber is in contact at a rate such that the fiber contacting surface is maintained at least 5° C. below the fusion temperature of the fiber at such contacting points to a final surface temperature between 135° C. and 190° C. and until said fibers have a residual solvent content of less than about 2 percent by weight and a fusion temperature of at least 150° C.

10 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9

ments and yarns having low solvent content from a vinyl polymer containing between about 40 percent and about 75 percent acrylonitrile polymerized therein, which includes the steps of extruding a dope consisting of the said polymer dissolved in a spinning solvent boiling below about 100° C. through a spinneret to form fibers containing less than about 20 percent by weight of residual solvent, and subjecting the formed fibers to direct contact with a heated surface maintained at a temperature of at least about 60° C. and between 5° C. and 20° C. below the fusion temperature of the fiber at the point of contact with the heated surface, increasing the temperature of the surface to which the fiber is in contact at a rate such that the fiber contacting surface is always maintained at least 5° C. below the fusion temperature of the fiber at such contacting points to a final surface temperature between 135° C. and 190° C. until said fibers have a residual solvent content of less than about 2 percent by weight and a fusion temperature of at least 150° C., and the total residence time of said fibers during the heating being 3 minutes or less, and thereby avoiding filament fusion and adhesion.

6. A process for continuously producing textile filaments and yarns having low solvent content free from interfiber fusion from a vinyl polymer in which at least one component is acrylonitrile present in a significant amount polymerized therein, which includes the steps of extruding a dope consisting of the said polymer dissolved in a spinning solvent boiling below about 100° C. through a spinneret to form fibers containing less than about 20 percent by weight of residual solvent and subjecting the formed fibers to direct contact with a heated godet having a temperature gradient maintained along the axial length of the circumferential surface of the godet, contacting the formed fibers with the cooler end of the godet maintained at a temperature of at least about 60° C. and between 5° C. and 20° C. below the fusion temperature of the fiber at the point of contact with the heated surface, advancing the fiber on the godet toward the hotter end such that the temperature of the fiber contacting surface is maintained at least 5° C. below the fusion temperature of the fiber to a final surface temperature between 135° C. and 190° C. until said fibers have a residual solvent content of less than 2 percent by weight and a fusion temperature of at least 150° C., thereby avoiding filament fusion and adhesion.

7. A process for continuously removing solvent from textile filaments and yarns of a vinyl polymer in which at least one component is acrylonitrile present in a significant amount polymerized therein and containing between 2 and 20 percent by weight of a solvent having an atmospheric boiling point below about 100° C., which includes the step of contacting the fiber first to a temperature of at least about 60° C. and between 5° C. and 20° C. below the fusion temperature of the fiber, increasing by increments the temperature to which the fiber is in contact to a final temperature between 135° C. and 190° C. at a rate such that the temperature to which the

fiber is in contact is always maintained at least 5° C. below the fusion temperature of the fiber at such points and until said fibers have residual solvent content of less than about 2 percent by weight and a fusion temperature of at least 150° C.

8. A process for continuously removing solvent from textile filaments and yarns of a vinyl polymer containing between about 40 percent and about 75 percent acrylonitrile polymerized therein and which contains from 2 to 10 percent by weight of a solvent having an atmospheric boiling point below about 100° C. which includes the step of subjecting the formed fibers to direct contact with a plurality of heated rolls in series, the first contacting roll being maintained at a temperature of at least about 60° C. and between 5° C. and 20° C. below the fusion temperature of the fiber at the point of contact with the heated surface, increasing by increments the surface temperature of the rolls to which the fiber is in contact at a rate such that the fiber contacting surface is maintained at least 5° C. below the fusion temperature of the fiber at such contacting points to a final surface temperature between 135° C. and 190° C. until said fibers have a residual solvent content of less than 2 percent by weight and a fusion temperature of at least 150° C.

9. A process for continuously removing solvent from textile filaments and yarns of a vinyl polymer containing between about 40 percent and about 75 percent acrylonitrile polymerized therein and which contains from 2 to 20 percent of a solvent having an atmospheric boiling point below about 100° C. which includes the step of subjecting the formed fibers to direct contact with a heated godet having a temperature gradient maintained along the axial length of the circumferential surface of the godet, contacting the formed fibers first with the cooler end of the godet maintained at a temperature of at least about 60° C. and between 5° C. and 20° C. below the fusion temperature of the fiber at the point of contact with the heated surface, advancing the fiber on the godet toward the hotter end such that the temperature of the fiber contacting surface is maintained at least 5° C. below the fusion temperature of the fiber to a final surface temperature between 135° C. and 190° C. until said fibers have a residual solvent content of less than 2 percent by weight and a fusion temperature of at least 150° C.

45

50

40

35

30

25

20

15

10

5

55

#### References Cited in the file of this patent

#### UNITED STATES PATENTS

|           |                     |               |
|-----------|---------------------|---------------|
| 2,244,745 | Uytenbogaart et al. | June 10, 1941 |
| 2,622,182 | Forzley et al.      | Dec. 16, 1952 |
| 2,692,185 | Hooper              | Oct. 19, 1954 |
| 2,697,023 | Martin              | Dec. 14, 1954 |
| 2,733,121 | Griffith            | Jan. 31, 1956 |
| 2,811,409 | Clapp               | Oct. 29, 1957 |

#### OTHER REFERENCES

Dupont Textile Fibers, Technical Information, Bulletin, July 1955.